

## UNITED STATES PATENT OFFICE.

RALPH E. SAYRE, OF MOUNT VERNON, NEW YORK, ASSIGNOR TO METALS RECOVERY COMPANY, OF NEW YORK, N. Y., A CORPORATION OF MAINE.

## CONCENTRATION OF ORES BY FROTH FLOTATION.

No Drawing.

Application filed May 11, 1928. Serial No 277,097.

This invention relates to the concentration of minerals, and has for its object the provision of certain improvements in the concentration of minerals by flotation. The invention more particularly relates to the concentration of minerals by froth flotation. Various organic mineral collecting agents have been proposed for the purpose of floating mineral particles, as distinguished from gangue particles, in froth flotation processes. They have met with varying degrees of success in commercial practice. Some of these agents are effective with certain ores, but yield relatively poor results with other ores. In general these agents may be employed in small amounts, but their cost of manufacture is frequently so high as to make their use uneconomical. It is therefore seen that, even though considerable progress has been made in the art of flotation agents, a wide field of application remains for an agent that is not only relatively cheap to make, but which can be used with a greater variety of ores to effect still higher recoveries of the valuable minerals.

The present invention is based on my discovery that organic selenium compounds are very effective mineral-collecting agents, particularly in the concentration of minerals by froth flotation. The invention accordingly comprises conducting the flotation operation in the presence of an organic selenium compound as the mineral-collecting agent. Among the organic selenium compounds that lend themselves to the practice of the invention may be mentioned such compounds as seleno-benz-amide ( $C_6H_5CSeNH_2$ ), ethyl-selenide ( $C_2H_5)_2Se$ , selenocarbanilid, or di-phenylselenourea ( $C_6H_5NH)_2CSe$ , phenyl-selenouethane  $C_6H_5NHSeOC_2H_5$ , seleno-phenol ( $C_6H_5SeH$ ) and its homologs, particularly selenocresol  $C_6H_4CH_3SeH$ .

The organic selenium compounds employed in the practice of the invention are essentially mineral-collecting agents and are substantially devoid of frothing power. In the concentration of minerals by froth flotation, employing such organic selenium compounds as mineral-collecting agents, it is therefore necessary to use a frothing agent, such as pine

oil, terpineol, cresol, aldol, or the like, to produce the necessary frothing action.

The organic selenium compound may be introduced into the ore or mineral pulp in any convenient manner and at any appropriate stage preceding or during the flotation operation. Thus, it may advantageously be ground with the ore, or it may be added to the comminuted ore at any stage prior to the flotation operation. The organic selenium compounds characteristic of the invention are sufficiently soluble in water so that they may be added to the pulp in solid form, preferably in a relatively fine state of subdivision. In order to secure prompt dissemination throughout the mineral pulp, the organic selenium compound may be dissolved in an appropriate solvent therefor and the resulting solution added to the pulp. The frothing agent is preferably, though not necessarily, added to the mineral pulp as the pulp enters the flotation apparatus. In certain cases it is advantageous to dissolve the organic selenium compound in the frothing agent, and then add the resulting solution to the pulp at any appropriate stage preceding or during the flotation operation.

The quantity of the organic selenium compound to be employed in practicing the invention depends to some extent on the ore or mineral being treated. Good results are attained with one pound, and less, of the organic selenium compound per ton of dry ore. In general, however, I have found that one-half of a pound, and less, per ton of dry ore gives satisfactory results.

While, in practicing the invention, the organic selenium compound may be used in an acid or neutral mineral pulp, I prefer to have the pulp slightly alkaline. Any alkali, such as caustic soda, soda ash, lime, or the like, may be added to the mineral pulp to make it neutral or alkaline. Lime, on the whole, is the most suitable and available alkali for this purpose. The alkali is preferably added to the mineral pulp before the final grinding, and before adding the organic selenium compound.

The following example is illustrative of the practice of the invention on Utah cop-

per ore, using seleno-benz-amide as the mineral collecting agent. The amounts of reagents specified are in terms of pounds per ton of dry ore:

| Reagents            | Amounts           |
|---------------------|-------------------|
| Seleno-benz-amide   | 0.44              |
| Frothing (pine oil) | 0.254             |
| Alkali (NaOH)       | 4.003             |
| Concentrates        | Per cent Cu.      |
| Concentrates        | 14.6              |
| Tailings            | 0.21              |
| Tailings            | Per cent recovery |
|                     | 72.8              |

My studies of the organic selenium compounds available for the practice of the invention have led me to the belief that their effectiveness in froth flotation processes is in large part due to the presence in the compound of selenium in a negative state and in a relatively low state of valence. In these organic compounds, the selenium is present as a di-valent negative element. The mineral-collecting agents of the present invention are therefore characterized by their reduced or di-valent negative selenium. In addition, the organic selenium compounds of the invention, like other organic non-oleaginous mineral-collecting agents, should impart to the mineral particle, when adsorbed or otherwise attached thereto, a water-repellent surface.

It is, of course, not necessary that substantially pure organic selenium compounds be employed in the practice of the invention, although more uniform and satisfactory results will be attained and better control of the selective action of the mineral-collecting agent is possible with commercially or practically pure organic compounds of selenium. However, commercial products and crude reaction products containing substantial and effective amounts of one or more organic selenium compounds may be used in carrying out the invention.

It will be understood by those skilled in the art that the present invention is applicable to the treatment of flotation of various kinds of mineral mixtures both natural and artificial. In the appended claims, I have accordingly employed the term "mineral"

in a broad sense to include ores, mineral products and all materials amenable to concentration or similar treatment by the flotation processes.

I claim:

1. The improvement in the concentration of minerals by froth flotation which comprises subjecting the mineral in the form of a pulp to a froth flotation operation in the presence of a mineral-collecting agent which is an organic selenium compound in which the selenium is present in a negative state.

2. The improvement in the concentration of minerals by froth flotation which comprises subjecting the mineral in the form of a pulp to a froth flotation operation in the presence of a mineral-collecting agent which is an organic selenium compound in which the selenium is present in a di-valent negative state.

3. The improvement in the concentration of minerals by froth flotation which comprises subjecting the mineral in the form of a pulp to a froth flotation operation in the presence of a mineral-collecting agent which is an organic selenium compound capable of imparting a water-repellent surface to mineral particles and in which the selenium is present in a di-valent negative state.

4. The improvement in the concentration of minerals by froth flotation which comprises subjecting the mineral in the form of a pulp to a froth flotation operation in the presence of seleno-benz-amide.

5. The improvement in the concentration of minerals by froth flotation which comprises subjecting the mineral in the form of a pulp to a flotation operation in the presence of a mineral-collecting agent which is an organic compound containing selenium chemically combined therewith.

6. The improvement in the concentration of minerals by froth flotation which comprises subjecting the mineral in the form of a pulp to a froth flotation operation in the presence of a mineral-collecting agent which is an aromatic compound containing selenium chemically combined therewith.

In testimony whereof I affix my signature.

RALPH E. SAYRE.